

# UNITED STATES PATENT OFFICE.

ALFRED WELLS CASE, OF HIGHLAND PARK, CONNECTICUT.

## MANUFACTURED LEATHER.

No. 878,485.

Specification of Letters Patent.

Patented Feb. 4, 1908.

Application filed February 7, 1907. Serial No. 356,155.

*To all whom it may concern:*

Be it known that I, ALFRED WELLS CASE, a citizen of the United States, and a resident of Highland Park, in the county of Hartford, 5 and State of Connecticut, have invented a new and Improved Manufactured Leather, of which the following is a specification.

My invention relates to the manufacture of comparatively thick sheets of material 10 from fiber, and more particularly to such sheets as are partially or wholly formed from animal fiber.

The object of the invention is the production of a piece or sheet of such material that 15 shall possess throughout the entire mass properties of consistency or density which are material in the articles usually produced from such sheets; and a further object of the invention is to provide means for properly stiffening sheets or pieces of such material to the required degree and maintain them in this condition until such time as they may be required for use for manufacturing purposes; and a further object of the 20 invention is to give to such sheets properties which will enable a nice finish to be given to the articles made therefrom.

In the manufacture of sheets of comparatively thick material from fiber, and more 30 especially that class commonly known as leather board, the leather scrap or like material, either alone or mixed with other fibrous matter, is reduced to pulp by a beating engine or the like, which by well-known treatment 35 is formed into sheets or board of the desired thickness. The sheets are then suitably dried as by the action of the elements, or by artificial means. In using the board for manufacturing purposes it is desirable 40 that the sheets shall have considerable density and consistency and shall have within certain well defined limits proper qualities as to stiffness. It is also desirable to give to articles formed therefrom a certain degree of 45 finish, and as such articles are, in many instances, formed from superimposed layers or pieces of material, the edges of which form the surface of the finished article it is evident that such material shall possess 50 throughout the entire thickness of the mass qualities to enable the articles made therefrom to take the desired finish, and to produce the best results that the qualities as to density and consistency shall be present 55 throughout the entire mass.

I have found by extended experiment that

rosin, if properly distributed throughout the mass, will give the board proper qualities as to density and consistency and also as to stiffness, and will also produce an article 60 which will receive a nice finish; how to properly introduce the rosin into the mass, however, has been a problem.

The rosin can not be introduced to the pulp for the reason that it not only gums up 65 the machinery to such an extent as to practically prevent its operation, but the rosin thus introduced will be in granulated form, which, upon melting, under the heat to which the sheets must subsequently be subjected leaves cells throughout the mass formerly occupied by the grains of the rosin. This forms a cellular mass which is extremely 70 objectionable. If the rosin is melted and the sheets immersed in a bath it is found that the 75 rosin chills so quickly as to that part in contact with the sheet that it permeates but very little if at all into the sheet. The rosin mixed with other materials has been applied to the sheets as a size, but it has been found 80 that such treatment produces little, if any, effect in causing the rosin to penetrate the fiber. After extended experiment I have found, however, that a liquid composed of a 85 greasy or oily substance, as wax or mineral oil, either or both, mixed with the rosin, heated to the proper degree and applied to the sheets will produce most beneficial results. The rosin is reduced to a liquid state by the 90 heat and the added matter acts not only as a vehicle to convey the rosin throughout the entire mass, but maintains the rosin in a liquid state and prevents such chilling as to cause the rosin to assume granular form.

The rosin, in addition to giving the qualities above described to the sheets of material, also acts to a certain extent as a water-proofing substance, and its mixture with the mineral oil or wax, or both, thoroughly water-proofs the sheets and preserves them in a 100 pliable state, while maintaining the required density and stiffness for indefinite lengths of time and until required for manufacturing purposes.

I have found that very beneficial results 105 are obtained in a bath heated to about 180 degrees. The proportions of the wax or mineral oil may be varied to any extent, and, in fact, wax alone or mineral oil alone may be mixed with the rosin and produce satisfactory results. The higher the proportion of wax to the mineral oil the better will be the

grade of the leather board. Sheets treated with mineral oil and rosin alone supply a large demand for certain classes of work, and hence it will be obvious that the better the 5 grade of work required the more wax in proportion to the mineral oil should be used. The proportion of the rosin may be varied almost indefinitely, depending upon the degree of finish required or the amount of density or consistency desired.

In making the mixture the mineral oil is employed as an element for the reason that the rosin and wax will be retained in the manufactured article under certain conditions as to temperature, whereas if vegetable or animal oils are employed the rosin and wax will ooze from the manufactured article under the application of lower degrees of temperature.

20 While I have found oil or wax to possess the necessary greasy or oily properties, and

also the necessary penetrating properties to produce excellent results, yet it is obvious that other greasy or oily substances may be employed, and as these materials resist the 25 entrance of water into the sheets of fiber board described herein I have termed the material used with the rosin a water resist, this including any greasy or oily substance which will serve the desired end. 30

What I claim as my invention and desire to secure by Letters Patent is:—

As an improved article of manufacture, a sheet of leather board formed from leather pulp material and after being formed and 35 dried treated to a bath including rosin and heated mineral oil.

#### ALFRED WELLS CASE.

Witnesses:

ARTHUR B. JENKINS,  
LENA E. BERKOVITCH.